

# UNITED STATES PATENT OFFICE.

FRANCIS C. FRARY, OF NIAGARA FALLS, NEW YORK, AND STERLING N. TEMPLE, OF ST. PAUL, MINNESOTA.

## COMPOSITION OF COPPER ALLOYS CONTAINING STRONTIUM.

1,258,886.

Specification of Letters Patent. Patented Mar. 12, 1918.

No Drawing.

Application filed March 31, 1916. Serial No. 87,990.

*To all whom it may concern:*

Be it known that we, FRANCIS C. FRARY and STERLING N. TEMPLE, citizens of the United States, and residents, respectively, of 5 Niagara Falls, in the county of Niagara and State of New York, and St. Paul, in the county of Ramsey and State of Minnesota, have invented certain new and useful Improvements in the Composition of Copper 10 Alloys Containing Strontium, of which the following is a specification.

Our invention has for its object to provide an alloy of copper having certain desirable properties, particularly hardness and 15 freedom from blow-holes in castings.

In carrying out our invention, as generally disclosed in our U. S. Patent No. 1,169,392, of Jan. 25, 1916, we alloy with the copper a small amount of metallic strontium, where- 20 by the copper is hardened and all dissolved gases are removed, causing the metal to make castings free from blow-holes. If the amount of strontium is small, the electrical conductivity of the copper is not materially 25 changed. It is to be noted that this hardness is produced in the metal when cast and cooled in the ordinary way, without mechanical treatment such as hard-drawing, etc., but such mechanical treatment could 30 also be applied to the alloy if desired.

In carrying out our invention, we may prepare a strontium-copper alloy by electrolysis of fused strontium chlorid, or a mixture of this salt with other salts, using a 35 molten copper cathode. By this means we

have prepared such an alloy, and find it to have the properties stated, even when the amount of strontium is less than one per cent. It is obvious that we may also prepare the alloy by melting copper, and thereafter 40 adding metallic strontium, or an alloy containing strontium, to the copper.

In the practical operation of our invention, we prefer to use with the strontium some other metal or metals of the alkaline 45 earths, as described in our U. S. Patent afore-mentioned, because we find that, in general, the presence of more than one of these elements increases the hardening effect of each, and because others, notably calcium, 50 are cheaper to prepare.

What we claim is:

As a new composition of matter, a metallic alloy harder than pure copper, containing a main body of copper, and in addition 55 thereto containing a small amount of strontium.

Signed at Niagara Falls, New York, this 28 day of March, 1916.

FRANCIS C. FRARY.

In presence of—

F. A. SCHUMACHER,  
T. A. STAMPS.

Signed at Keokuk, Iowa, this 24th day of March, 1916.

STERLING N. TEMPLE.

In presence of—

J. F. REIDY,  
ARNOLD MOHN.